

Sept. 12, 1944.

G. L. BOULET

2,358,050

METHOD AND APPARATUS FOR MANUFACTURING AND CONTROLLING  
THE GRAIN SIZE OF BARIUM SULPHATE

Filed Dec. 6, 1941



Gerald L. Boulet  
INVENTOR

BY *Merton M. Purvis*  
*Jack T. Harrington*  
ATTORNEYS

## UNITED STATES PATENT OFFICE

2,358,050

## METHOD AND APPARATUS FOR MANUFACTURING AND CONTROLLING THE GRAIN SIZE OF BARIUM SULPHATE

Gerald L. Boulet, Rochester, N. Y., assignor to Eastman Kodak Company, Rochester, N. Y., a corporation of New Jersey

Application December 6, 1941, Serial No. 421,978

7 Claims. (Cl. 23—122)

The present invention relates to the manufacture of precipitated barium sulphate (*blanc fixe*), and particularly to the control of the grain size of the precipitate.

Precipitated barium sulphate has many uses, but the one which is primarily of interest in connection with the present invention is its use as a coating for photographic papers. In the manufacture of barium sulphate for coating photographic papers, it is necessary to control the grain size very closely depending upon the finish desired on the paper. It has been found that a fine-grain size barium sulphate imparts a relatively high gloss to processed paper, while the larger grain size material results in a surface that is dull, even to a matte finish.

In large scale production, precipitated barium sulphate is usually made by mixing a soluble sulphate solution with a soluble barium salt. There are several known methods of controlling the grain size of the precipitate including, varying the concentration of the solutions, varying the temperature of the solutions, and varying the speed of stirring or agitation at the time of contact of the solutions. Any, or all, of the above-mentioned factors can be adjusted to meet certain conditions very nicely, but there are times, especially in large scale manufacture control, where more flexibility is desirable. Also, if, during the manufacture of the precipitate, any one of the above variables should get out of control it is desirable to be able to compensate for it with a minimum of cost and inconvenience.

Therefore, the primary object of the present invention is the provision of a method and apparatus for manufacturing precipitated barium sulphate by which the grain size of the precipitate can be readily controlled by merely varying the relative points of introduction of the solution into the precipitating chamber.

Another object is the provision of a method and apparatus by means of which changes in grain size of the precipitate due to variations in temperature of the solutions, concentration of the solutions, etc., can be readily accounted for in a rapid and efficient manner by a mere mechanical adjustment at the precipitating chamber.

The novel features that I consider characteristic of my invention are set forth with particularity in the appended claims. The invention itself, however, both as to its organization and its methods of operation, together with additional objects and advantages thereof, will best be understood from the following description of

specific embodiments when read in connection with the accompanying drawing in which,

Fig. 1 is a sectional view of one form of apparatus constructed in accordance with the present invention,

Fig. 2 is a top plan view of the apparatus shown in Fig. 1, and clearly showing the manner of adjusting the position of the conduits toward and from the center of the precipitating chamber,

Fig. 3 is a plan view showing a modified form of conduit supporting and adjusting mechanism, and

Fig. 4 is an elevational view of a standard settling tube which can be used in determining the grain size of the precipitated barium sulphate.

Like reference characters refer to corresponding parts throughout the drawing.

Briefly, in accordance with the present invention a barium salt solution and a soluble sulphate solution are continuously introduced into a precipitating chamber where they are mixed together due to the action of an agitator, or stirrer, in the chamber. The two solutions are introduced into the precipitating chamber on opposite sides of the center thereof and the points of introduction of the two solutions are adjusted to and from the center of the chamber to vary the grain size of the precipitate.

In accordance with the present invention, precipitated barium sulphate (*blanc fixe*) is manufactured by introducing a barium sulphate solution from a storage tank 10 and a soluble sulphate solution from a storage tank 11 continuously into a precipitating chamber 12. This precipitating chamber may be an open ended earthen-ware tile, as shown in Fig. 1, vertically disposed in an earthen ware receptacle 13. Extending into the center of the open end of the precipitating chamber 12 is a shaft 8 on the end of which there is an impeller, or agitator, 14 which may be driven by any suitable means, such as motor M. The lower end of the precipitating chamber 12 is spaced from the bottom of the receptacle 13 by a foot 15 formed on the end of the tile so that the precipitate formed in the chamber 12 can flow out of the bottom of the tile and into the receptacle 13, as indicated by the flow arrows. It will be noticed that the upper end of the chamber 12 is above the upper edge of the receptacle 13 so that the barium sulphate will continually flow from the chamber 12 into the receptacle 13 and spill over the top thereof. This overflow of barium sulphate precipitate will be caught in a pan 8 and conducted

30

35

40

45

50

55

to a settling tank, not shown, where the precipitate can settle from the liquid.

The solutions are conducted from the storage tanks 10 and 11 through pipes 16 and 17, respectively, into conduits 18 and 19 adjustably mounted on a support 20 extending diametrically across the upper end of the precipitating chamber 12. Conduits 18 and 19 may be of any suitable shape so long as they serve to collect the solutions from the pipes and discharge them into the chamber, and for the purposes of illustration, I have shown them as funnels the outlets 21, 22 of which discharge the solutions into the chamber 12. The conduit 18 for the barium salt solution is mounted on one side of the center of the chamber 12 and the conduit 19 for the soluble sulphate solution is mounted on the opposite side of the center of the chamber.

I have found that the grain size of the barium sulfate precipitate can be easily and efficiently controlled by moving the two conduits 18 and 19 toward and from the center of the chamber, and for this reason the conduits are supported so that they can be adjusted to and from the center of the chamber. As shown in Fig. 1, the support 20 may be provided with a plurality of apertures 26 located on opposite sides of the center of the chamber from one to the other of which the conduits 18 and 19 can be shifted on their respective sides of the chamber to vary the grain size.

I have found that with both solutions entering at the closest position to the center of the chamber, the resulting grain size is as fine as possible with the particular solutions being used. Likewise, when the solutions are introduced into the precipitating chamber at the wall position on opposite sides of the center of the chamber, the resulting grain size is as large as possible with the solutions in use. Introducing the solutions at intermediate distances results in grain sizes between the above-mentioned fine grain and large grain.

I have found barium chloride ( $BaCl_2$ ) and sodium sulphate ( $Na_2SO_4$ ) to be very satisfactory compounds for forming the solutions necessary to the manufacture of precipitated barium sulphate on a large scale primarily because each of these compounds is readily obtained at a reasonable price and they combine to form a solution of sodium chloride which can be easily washed from the final barium sulphate precipitate. However, it is pointed out that the invention is not limited to the compounds specified, but covers the use of any soluble barium salt and soluble sulphate. I have also found that a solution of 4000 pounds of barium chloride and 2600 pounds of sodium sulphate each dissolved in 3000 gallons of water, when mixed in the manner set forth, combine to form a very good yield of precipitated barium sulfate of good quality.

Determination of the grain size of barium sulphate can be carried out in several different ways. The method which I have found to be particularly adapted for use in manufacturing and production control because of the ease and rapidity with which it can be carried out is described below. The solution containing the barium sulphate to be measured is introduced into a standard 250 cc. settling tube 27, as shown in Fig. 4, to the upper 0-250 cc. mark. The neck of the tube is then closed with a ground glass stopper 28 and the contents thoroughly mixed by inverting the tube several times. The tube is then placed on a solid support and the time noted. After ten minutes the precipitate will have settled downwardly

and the reading is taken at the point to which the precipitate has settled in that time, reading the descending rather than the ascending scale. Actually the tube is calibrated in 2 cc. steps so that it can be read quite accurately, while I have shown only 25 cc. steps for purposes of clarity. By microscopic measurement it has been found that a sample that settles 36 cc. in ten minutes had a grain size of .25 mu, while one that settled only 15 cc. in ten minutes measures .15 mu by the same method.

The following table shows the results of two test runs which prove that the grain size of the barium precipitate can be altered by changing the positions of the point of the introduction of the two solutions into the precipitating chamber. The solutions used in the following tests were a barium chloride solution and a sodium sulphate solution of a given concentration using a settling time of ten minutes.

| Outer position | Intermediate position | Innermost position |
|----------------|-----------------------|--------------------|
| Cc.            | Cc.                   | Cc.                |
| 86<br>88       | 66<br>50              | 6<br>10            |

The above table shows that when the two solutions were introduced at the most extreme position from the center of the precipitating chamber that more precipitate settled in a given time than when introduced at positions closer to the center of the chamber. Since the amount of precipitate settled in a given time is a direct indication of the grain size of the precipitate, as set forth above in describing the settling test for determining the grain size, it will be obvious that the grain size changes from a maximum to a minimum as the solutions are introduced nearer to the center of the precipitating chamber. A larger precipitating chamber or less concentrated solutions will give a wider range, while a smaller chamber or more concentrated solutions will shorten the range of grain sizes producible.

I realize that it is not necessary to use the identical apparatus as set forth to obtain the same ends. Any similar set-up that would allow the solutions to mix in the manner above described, and any device that would permit the points of introduction of the solutions into the precipitating chamber to be adjusted to and from the center of the precipitating chamber so as to result in the above-mentioned grain size control, would come within the scope of the present invention. By way of example of another modification in the apparatus which would be suitable for carrying out the present invention, I have shown in Fig. 3 another manner in which the conduits for the solutions could be mounted on the top of the chamber to facilitate their adjustment to and from the center of the chamber. As shown in Fig. 3, the conduit 18' could be fixed to a slide 36 slidably mounted on rails 37 extending longitudinally of a support 20' having a slot 38 extending lengthwise thereof through which the outlet of the conduit extends into the chamber 12. Slide 36 is adapted to be nicely adjusted toward and from the center of the chamber along the support 20' by adjustment of a hand screw 39 engaging a threaded eye 40 fixed to the slide. Instead of having the conduits 18 and 19 in the form of funnels having the mouths large enough to catch the flow from the pipes 16 and 17 in any position of ad-

justment, it will be obvious that the pipes could be made flexible and have their ends directly connected to a conduit movable along the support 20 to permit them to be adjusted to and from the center of the chamber to control the grain size of the precipitate.

It is acknowledged that it might be possible to accomplish the control of grain size of the precipitated barium sulphate by controlling the stirrer speed, but such a method of control in a manufacturing set-up is rather inconvenient. Temperature adjustments probably would do the same thing, but that also would be inconvenient for the reason that it would be slow and difficult to closely regulate. Varying the concentration of the solutions also might do it, but here also it would be impractical and inconvenient in a manufacturing set-up for large scale production. From the above description it will be readily apparent to one skilled in the art that by the use of the herein disclosed method and apparatus the grain size of precipitated barium sulphate can be readily controlled over a substantially wide range by a mere mechanical adjustment of the apparatus and a change in grain size can, therefore, be accomplished quickly and efficiently by an unskilled operator. Furthermore, by the use of this method of grain size control any change in the desired grain size due to variations in the temperatures of the solutions, concentration of the solutions or for other unforeseen reasons, can be quickly and easily accounted for by merely adjusting the point of introduction of the solutions into the precipitating chamber to correct for such variation. The method is so simple that any existing apparatus could be readily changed in view of the teachings of this disclosure to carry it out in the manner set forth.

Although I have shown and described certain specific embodiments of my invention, I am fully aware that many modifications thereof are possible. My invention therefore is not to be restricted except insofar as is necessitated by the scope of the appended claims.

Having thus described my invention, what I claim as new and desire to secure by Letters Patent of the United States is:

1. In a method of making barium sulphate and controlling the grain size thereof the steps of selecting a predetermined grain size for the barium sulphate, continuously introducing a barium salt solution and a soluble sulphate solution into an enclosure at separated points and agitating the solutions within the enclosure, determining the grain size of the barium sulphate formed and comparing it with the predetermined grain size and noting the difference between the two, and then moving the points of introduction of the two solutions toward and away from one another until the predetermined grain size is obtained, the grain size varying in direct proportion with the variation in the spacing of the points of introduction of the two solutions relative to one another.

2. In a method of making barium sulphate and controlling the grain size thereof the steps of selecting a predetermined grain size for the barium sulphate, continuously introducing a barium salt solution and a soluble sulphate solution into an enclosure at separated points on opposite sides of the center of the enclosure, and agitating the solutions within the enclosure with a circular motion, determining the grain size of

the barium sulphate formed and comparing it with the predetermined grain size and noting the difference between the two, and then moving the points of introduction of the solutions toward and away from one another during the production run until the selected predetermined grain size is obtained, the grain size varying in direct proportion with the variation in the spacing of the points of introduction relative to one another, other conditions being maintained unchanged.

3. In a method of making barium sulphate and controlling the grain size thereof the steps of selecting a predetermined grain size for the barium sulphate, continuously introducing a barium chloride solution and a sodium sulphate solution into an enclosure at separated points, continuously agitating the solutions within the enclosure so as to mix the two together, determining the grain size of the barium sulphate formed and comparing it with the predetermined grain size and noting the difference between the two, and then moving the points of introduction of the two solutions relative to one another to vary the spacing therebetween until the predetermined grain size is obtained, the grain size varying in direct proportion with the variation in the spacing of the points of introduction of the two solutions relative to one another, other conditions being maintained unchanged.

4. A method of making precipitated barium sulphate and controlling the grain size thereof comprising the steps of selecting a predetermined grain size for the barium sulphate, continually introducing a barium chloride solution containing 4000 lbs. of barium chloride and a sodium sulphate solution containing 2600 lbs. of sodium sulphate into an enclosure at separated points on opposite sides of the center of the enclosure, agitating the solutions within the enclosure with a circular motion about the center of the enclosure, determining the grain size of the barium sulphate formed and comparing it with the predetermined grain size and noting the difference between the two, and then moving the points of introduction of the two solutions toward and away from the center of the enclosure during the production run until the predetermined grain size is obtained, the grain size varying in direct proportion with the variation in the spacing of the points of introduction of the solutions relative to one another, other conditions being maintained unchanged.

5. In a method of making barium sulphate and controlling the grain size thereof the steps of continuously introducing a barium salt solution and a soluble sulphate solution into an enclosure at separated points, agitating the solutions within the enclosure, determining the grain size of the barium sulphate produced, selecting a predetermined grain size smaller than that produced, and moving the points of introduction of the two solutions toward one another until the predetermined selected grain size is obtained, other conditions being maintained unchanged.

6. In a method of making barium sulphate and controlling the grain size thereof the steps of continuously introducing a barium salt solution and a soluble sulphate solution into an enclosure at separated points, agitating the solutions within the enclosure, determining the grain size of the barium sulphate produced, selecting a predetermined grain size larger than that produced, and adjusting the points of introduction

of the two solutions away from one another until the predetermined selected grain size is obtained, other conditions being maintained unchanged.

7. An apparatus for carrying out reactions involving the formation of a precipitate and controlling the grain size thereof, comprising a vertically disposed open-ended circular precipitating chamber, a support extending across the upper end of said chamber and provided with a plurality of apertures extending along said support 10

on each side of the center thereof, the order of spacing of said apertures being the same on each side of the center of the support, a pair of liquid receiving means removably supported in the apertures of said support, at least two sources of supply of reacting solution, pipe means connected to said sources of supply and associated with said liquid receiving means and agitating means in said chamber.

GERALD L. BOULET.